

April 4, 1950

J. J. A. P. VAN AMSTEL  
METHOD OF MANUFACTURING BLOCKING-LAYER  
CELLS OF THE SELENIUM TYPE  
Filed Sept. 21, 1945

2,502,540



Fig. 1.



Fig. 2.

## UNITED STATES PATENT OFFICE

2,502,540

## METHOD OF MANUFACTURING BLOCKING-LAYER CELLS OF THE SELENIUM TYPE

Johannes Jacobus Asuerus Ploos van Amstel,  
Eindhoven, Netherlands, assignor to Hartford  
National Bank & Trust Co., Hartford, Conn.,  
as trustee

Application September 21, 1945, Serial No. 617,917  
In the Netherlands February 22, 1943

Section 1, Public Law 690, August 8, 1946  
Patent expires February 22, 1963

5 Claims. (Cl. 175—366)

1

This invention relates to a method of manufacturing blocking-layer cells of the selenium type, particularly measuring rectifiers, in which a carrier plate has mounted on it a semi-conductive and a good conducting electrode. The semi-conductive electrode may be made for example of selenium, the good conducting one of gold. The two electrodes are generally assumed to be separated by a blocking layer. It has been suggested before to mount a lacquer film upon such a cell after the good conducting electrode is placed in position, *inter alia* in order to protect this electrode from the action of the metal by means of which the current supply conductor was secured to the counter electrode as shown in my copending United States application, Ser. No. 617,578, now Patent No. 2,446,254, issued August 3, 1948.

When ascertaining the relation existing with rectifiers between the current transmitted in a forward direction and the voltage supplied, it is found that this current is comparatively lower at low voltages than at a higher voltage. When rectifying low voltages in general, this property is detrimental but particularly in the case of measuring rectifiers a higher forward current is frequently endeavoured to be obtained even if small voltages are supplied. The scale division of the measuring instrument is thus given a more linear character.

It has now been found that when in accordance with the invention in the manufacture of blocking-layer cells of the selenium type a lacquer layer is applied subsequent to the counter electrode being placed in position and the cell is subjected to a heating up to a temperature ranging between 120 and 200° C. a considerable improvement of the properties of the cell in the above-mentioned sense is obtained. Obviously, use should be made of a lacquer which is secure against the heating applied.

It is quite known *per se* and even the standard practice to immerse a rectifier in an anti-corrosive lacquer after the good conducting electrode is placed in position. In addition, after lacquering these rectifiers will generally be subjected to heating either deliberately in order to dry the lacquer or involuntarily while the rectifier is in use. This heating will, however, be limited to the usual maximum operating temperature which lies at about 65° C. Such a temperature and even a higher temperature of, say, 80° C. is not liable to bring about the effect achieved by the invention.

In a preferred embodiment of the invention heating is carried out at 170° C. for half an

2

hour. Neither the temperature nor the duration of the treatment are, however, critical.

In order that the invention may be clearly understood and readily carried into effect it will now be described more fully with reference to the accompanying drawing in which:

Fig. 1 is a curve illustrating the voltage-current relationships in two cells, one of which is provided with a baked lacquer coating.

Fig. 2 is a curve illustrating on a logarithmic scale the voltage-current relationship in two cells, in the region of low voltages, one of the cells being provided with a baked lacquer coating, and

Fig. 3 illustrates one embodiment of a blocking layer cell which has been provided with a lacquer coating which has been baked in air at an elevated temperature.

Referring more particularly to Fig. 3 of the drawing, a blocking layer cell constructed in accordance with the invention is illustrated. A carrier plate 10 of galvanized aluminum is coated with a film of carbon which for the sake of clarity in the drawing is not shown. A layer of selenium 11 is applied to the carrier plate by casting after which the selenium is converted into the semi-conducting modification by a heat treatment in a heated press. A blocking layer is then formed on the selenium layer which is extremely thin and is not illustrated in the drawing. A round gold electrode 12 having a diameter preferably between 1 and 3 mms. is applied to the selenium layer 11 by atomization of the gold after which the electrode assembly is sprayed with a solution of polystyrene. The polystyrene coating is baked in air at a temperature up to about 170° for half an hour forming a solid coating of polystyrene 13 around the electrode assembly. The supply conductor 15 is secured to a metallic contact 14 which has been applied to the polystyrene layer 13 for making electrical contact to the gold electrode 12. For the sake of convenience, the layer of polystyrene has been greatly exaggerated, and it will be clearly understood that in the actual construction of the cell the thickness of the polystyrene film is exceedingly thin.

The results are illustrated in the characteristic curves.

In the right-hand half of Fig. 1 is plotted the forward current relatively to the voltage applied. The curve A relates to the properties of a cell which has not been subjected to heating, the curve B relates to a cell made by the method of the invention. The return current is plotted in the left-hand half of Fig. 1, the scale being,

however, different from that in the right-hand half. It is clearly shown in this figure that the forward current increased, whereas the return current decreased.

In order better to bring out the differences in the region near the voltages of about 0.2 volt, Fig. 2 shows again the right-hand half of Fig. 1, the currents being now plotted on a logarithmic scale. It is obvious how the initial values are much higher with the curve B than with the curve A. It is this region which matters particularly with measuring rectifiers.

What I claim is:

1. The method of manufacturing a blocking layer cell comprising the steps of forming a semi-conductive electrode on a base, forming a blocking layer on said semi-conductive electrode, forming a conductive electrode on said blocking layer, applying a coating of lacquer to the electrode assembly, and baking the lacquer at a temperature between about 100° and 200° C. until the lacquer has dried.

2. The method of manufacturing a blocking layer cell comprising the steps of forming a layer of selenium on a base, converting the selenium to a semi-conductive modification thereof, forming a blocking layer on said selenium layer, forming a conductive electrode on said blocking layer, applying a coating of polystyrene to the electrode assembly, and baking the polystyrene in air at a temperature of between approximately 100 to 200° C. until the polystyrene has dried.

3. The method of manufacturing a blocking layer cell comprising the steps of, forming a layer of selenium on a base, converting the selenium to a semi-conductive modification thereof, forming a blocking layer on said selenium layer, form-

ing a conductive electrode on said blocking layer, applying a coating of polystyrene to the electrode assembly, and baking the polystyrene coating in air at a temperature of approximately 170° C. for approximately one half hour.

4. A blocking layer cell comprising a carrier plate, a semi-conductive electrode on said carrier plate, a blocking layer on said semi-conductive electrode, a conductive electrode on said blocking layer, and a coating of baked lacquer covering the electrode assembly.

5. A blocking layer cell comprising a carrier plate, a layer of selenium on said carrier plate, a blocking layer on said selenium layer, a conductive electrode of smaller cross-section than said selenium layer on said blocking layer, and a coating of baked polystyrene covering the electrode assembly.

JOHANNES JACOBUS ASUERUS  
PLOOS VAN AMSTEL.

#### REFERENCES CITED

The following references are of record in the file of this patent:

#### UNITED STATES PATENTS

| Number    | Name           | Date          |
|-----------|----------------|---------------|
| 1,932,067 | Duhme          | Oct. 24, 1933 |
| 2,134,131 | Kipphan        | Oct. 25, 1938 |
| 2,182,377 | Guanella       | Dec. 5, 1939  |
| 2,345,122 | Herrmann       | Mar. 28, 1944 |
| 2,419,602 | Skinker et al. | Apr. 29, 1947 |

#### OTHER REFERENCES

Transactions of the Electrochemical Society for 1945, pages 275-287.